

Patented Dec. 8, 1925.

1,564,689

# UNITED STATES PATENT OFFICE.

NEIL S. KOCHER AND VICTOR E. KIMMEL, OF ROCHESTER, NEW YORK, ASSIGNEES TO  
EASTMAN KODAK COMPANY, OF ROCHESTER, NEW YORK, A CORPORATION OF  
NEW YORK.

## METHOD OF REDUCING THE VISCOSITY CHARACTERISTICS OF NITROCELLULOSE.

No Drawing.

Application filed February 25, 1925. Serial No. 11,591.

*To all whom it may concern:*

Be it known that we, NEIL S. KOCHER and VICTOR E. KIMMEL, citizens of the United States of America, residing at Rochester, in 5 the county of Monroe and State of New York, have invented certain new and useful Improvements in Methods of Reducing the Viscosity Characteristics of Nitrocellulose, of which the following is a full, clear, and 10 exact specification.

This invention relates to processes for treating introcellulosic materials in order to lower the viscosity characteristics of the nitrocellulose. One object of the invention 15 is to provide a process for lowering the viscosity characteristics of the nitrocellulose, which will be safe, simple, and inexpensive. Another object of the invention is to provide such a process in which the treatment 20 will be under accurate control, and in which the results may, therefore, be readily duplicated. Still another object of the invention is to provide a process which may be carried out at atmospheric pressure without 25 the necessity of special pressure apparatus. Another object of the invention is to provide a process which may be carried out at room temperature within a reasonably short time without the expense and trouble of 30 heating operations. Other objects will hereinafter appear.

For certain purposes there is a demand for solutions of nitrocellulose which are concentrated and yet spray easily,—that 35 is, they have a high percentage of nitrocellulose in them, but have a low viscosity. The kinds of nitrocellulose which are met with most frequently have high viscosity characteristics, and can not be formed 40 into the above mentioned solutions without modification. Moreover, the kinds of nitrocellulose which are present in pyroxylin waste and film scrap or other sources of cheap waste material, have high viscosity 45 characteristics. It is, therefore, desirable to provide a safe, simple and cheap process for converting such high viscosity types of nitrocellulose into those of low viscosity characteristics, which can be used in the 50 above mentioned spraying operations.

We have found that the viscosity characteristics of nitrocellulosic material may be usefully lowered for this purpose, by treating it with an acid solution of a chlorate

of an alkali metal, such for example, as potassium chlorate. The treatment is preferably conducted at atmospheric pressure, and at room temperature. While heating will accelerate the action, it is preferable to proceed at room temperature, the action being 60 sufficiently rapid for practical purposes. This treatment is applicable to nitrocellulose in various forms, such as in the form of original nitrated cellulose fibers, or in the form of colloidized products such as solid 65 colloidized film scrap, and pyroxylin waste. The nitrocellulose may be associated or not with softeners or high-boiling organic compounds like camphor, butyl alcohol and etc. We shall now give a specific example of one 70 application of our process, but it will be understood that the invention is in no way restricted to the details thereof except as indicated in the appended claims.

The nitrocellulose material, such as pyroxylin waste, or film scrap from which the gelatinous coatings have been removed, is treated in a bath of strong mineral acid containing a small amount of potassium chlorate. The material is preferably comminuted so as to expose a large area, relative to its mass, thus promoting a uniform action throughout the whole of it. The pieces of material are preferably kept covered with the solution during the treatment. One 85 bath which we have found useful is an aqueous solution of hydrochloric acid containing approximately 36% of the latter, and also containing about one-tenth of one per cent of potassium chlorate. Another 90 equally suitable bath is a solution of nitric acid in water of approximately 65% strength, and likewise containing about one-tenth of one per cent of potassium or sodium chlorate.

The duration of the treatment varies, and the time to end it is preferably determined by tests. Representative samples of material are taken from time to time, washed, dried, and then dissolved in order to test 100 their viscosity characteristics. In general, the time of treatment will be decreased with increased concentration of acid, with increased concentration of the chlorate (within limits), by using nitrocellulose of medium viscosity characteristics at the start of the process, and by increasing the temperature of the bath. By accepting only a moderate

reduction in viscosity the process will likewise be shortened. Consequently, when working at room temperature, we may vary the duration of treatment from a few hours 5 to several days. In the above examples we may substitute original nitrated cotton fibers instead of colloidized nitrocellulosic materials. The concentrations of the acids may also be reduced, but we prefer to work with 10 strong solutions, as indicated above.

During the action, a mild denitration may take place, but the reduction in viscosity reaches the desired state before the denitration has proceeded to a harmful extent. In general we do not prefer to reduce 15 the percentage of the nitrogen in the nitrocellulose below 9.5%. When it proceeds much below this proportion, the solubility of the product in the usual solvents is seriously affected. 20

When the action of the bath is complete, it is drained off from the material, and the latter is fully washed. It may, for example, be treated with cold running water for 25 several days or even a week. Warm baths may be employed, say at 75° C. in order to remove the last traces of acid.

Having thus described our invention, what we claim as new and desire to secure 30 by Letters Patent is:

1. The process of treating nitrocellulosic material, which comprises acting thereon with a solution of mineral acid containing a chlorate of an alkali metal until the viscosity characteristics of the nitrocellulose are reduced, the action being stopped before denitration of the nitrocellulose reduces its 35 nitrogen content below 9.5%.

2. The process of treating nitrocellulosic material, which comprises acting thereon with a concentrated aqueous solution of mineral acid containing less than one per cent of chlorate of an alkali metal, until the viscosity characteristics of the nitrocellulose are reduced, the action being stopped before denitration reduces the percentage of 40 nitrogen in the nitrocellulose below 9.5%.

3. The process of treating nitrocellulosic material, which comprises acting thereon with a concentrated aqueous solution of 50 hydrochloric acid containing less than one per cent of potassium chlorate, the action being stopped before denitration impairs the solubility of the nitrocellulose.

4. The process of treating solid colloidal 55 nitrocellulose associated with a high-boiling organic compound, which comprises immersing said nitrocellulose in a bath containing a strong aqueous solution of mineral acid and potassium chlorate, the action being 60 stopped before denitration reduces the nitrogen in the nitrocellulose below 9.5%.

5. The process of treating solid colloidized nitrocellulose associated with a high-boiling organic compound, which comprises 65 immersing the same in a concentrated aqueous bath of mineral acid containing one-tenth of one per cent of potassium chlorate, the action being stopped before denitration reduces the percentage of nitrogen in the 70 nitrocellulose below 9.5%.

6. The process of treating nitrocellulosic materials containing nitrocellulose mixed with a high-boiling organic compound, which comprises immersing the same in a 75 bath containing a solution of mineral acid of more than 30% strength, said bath containing less than one per cent of the chlorate of an alkali metal, the action being stopped before the percentage of nitrogen is reduced 80 below 9.5% in the nitrocellulose.

7. The process of treating solid colloidized nitrocellulose which comprises acting on the same with 36% hydrochloric acid bath containing one-tenth of one per cent of potassium chlorate, the action being maintained until the viscosity characteristics of the nitrocellulose are reduced, but being stopped before the percentage of nitrogen in the nitrocellulose is reduced below 9.5%. 85 90

Signed at Rochester, New York, this 30th day of January, 1925.

NEIL S. KOCHER,  
VICTOR E. KIMMEL.